

Sept. 15, 1925.

1,553,646

F. THARALDSEN

PROCESS FOR THE PRODUCTION OF ZINC AND OTHER VOLATILE METALS

Filed Sept. 25, 1922.



Inventor

Philip Tharaldsen

By *Henry Ortho*  
Attn: my

Patented Sept. 15, 1925.

1,553,646

# UNITED STATES PATENT OFFICE.

FILIP THARALDSEN, OF BESTRUM, NEAR CHRISTIANIA, NORWAY.

## PROCESS FOR THE PRODUCTION OF ZINC AND OTHER VOLATILE METALS.

Application filed September 25, 1922. Serial No. 590,434.

*To all whom it may concern:*

Be it known that I, FILIP THARALDSEN, a citizen of Norway, residing at Bestrum, near Christiania, Norway, have invented certain new and useful Improvements in Processes for the Production of Zinc and Other Volatile Metals, of which the following is a specification.

When producing volatile metals by distillation, and specially when making zinc, it is known that the whole quantity of metal extracted is not obtained as pure metal in a molten state. In the case of zinc, a greater or smaller part of the extracted metal is obtained in form of blue powder, which in spite of its high contents of metal, of from 90 to 95% Zn., does not right away disengage fluid zinc at temperatures above the melting point of zinc.

Especially in the electrothermic manufacture of zinc, with the greater dimensions of the distillation chambers and the condensers necessary hereto, it has proved to be very difficult to keep the formation of blue powder within reasonable bounds, and no doubt it is owing to these difficulties that the electrothermic process has not attained the technical propagation, which its advantages compared with the old muffle process should justify.

The means hitherto employed to reduce the formation of blue powder in the electrothermic process have chiefly consisted in a mechanical treatment of the powder already formed, either in the condenser or after the removal from same, in order to make it yield part of its zinc contents as liquid metal. However, it is obvious that such methods are imperfect and only to be considered as makeshift while the difficulties presented by the formation of powder will only be really solved by avoiding as much as possible the conditions that lead to the said formation.

I have now ascertained that this can be attained by effecting the condensation of the metal vapours under the conditions described below.

In order to have a complete control of the temperature in the condenser this contains according to my invention always a fair-sized bath of metal over which the zinc vapours are passing. By reason of the great bulk of the bath the temperature varies very little. The temperature of the bath is kept at the most convenient height for the con-

densations by suitable cooling for instance by air or other gas. Cooled air of a convenient temperature can eventually be caused to pass through a mantle surrounding externally those surfaces of the condenser which internally are in touch with the metal bath. The temperature in the metal bath can be measured continuously by any suitable means and is kept constant by regulating the quantity, or the temperature, of the cooling medium. In order to obtain a constant temperature of condensation care must be taken that the condensation essentially takes place against the surface of the metal bath as cooling surface. To this effect the other surfaces of the condenser are kept at a temperature above the condensation point, which can be made by heat-insulating these parts of the condenser so well that only an insignificant quantity of heat dissipates.

It proves to be of great importance to avoid the formation of powder that the metal bath, on which the condensation takes place shall have a clean metallic surface, and means must therefore be provided for to remove during the operation an eventual film of oxide or a thin coating of powder, which may settle here. This can be done in different ways. A further quantity of molten zinc can for instance during work be supplied to the bath from outside whereby a current sets in on the surface of the bath towards the overflow. Through this movement of the surface of the bath the skin or the coating will move towards the overflow, and a bright surface of metal appears. It is also possible to remove the coating by means of suitable implements which are moved across the surface of the bath. It is understood that also other equivalent means may be used to keep the surface of the metal bright.

The annexed drawing illustrates diagrammatically a form of arrangements which can be used in carrying out the process.

Fig. 1 is a vertical section,

Fig. 2 a transverse section on the line 2—2 of Fig. 1.

From the furnace chamber A the zinc vapours pass into the condensation chamber B where they come in contact with the metal bath C at the bottom of the condenser and condense. Naturally this metal bath is established at the beginning of the process by introduction of molten zinc. As the condensation goes on, a corresponding quantity of

- metal passes over the overflow D down into the sump E, from where it can be drawn off. If desired, the condenser can be provided with several metal baths C and sums E in a row. In Fig. 1 are shown two of each. From the last metal bath the zinc vapours, which are now very poor in zinc, can pass out into the air through the opening G, eventually after having passed through a special reservoir first where the last parts of zinc are deposited as blue powder. The arrangement for cooling the metal bath consists of a plurality of flues J extending beneath the metal baths and provided with inlets and outlets  $j'$ ,  $j^2$  respectively for the passage of cooling air therethrough. For maintaining the temperature of the other surfaces of the condenser above the condensation point a covering B' of a suitable heat insulation material is spread over the top and sides of the condenser. H is the inlet for molten zinc to the metal bath C for charging or cleaning it.
- It will thus be seen that the stream of vapors enters one end of the furnace and passes over the several baths of molten zinc in succession and the condensation is facilitated by reason of the surface of the bath or baths being maintained unbroken.
- By not passing the zinc vapors through the body of the bath to cause it to bubble or causing the metal to drop or splash into the bath, the surface is kept substantially

continuous or unbroken whether there be surface movement or not and there is much less blue powder mixed in the bath. 35

I claim:

1. The process of condensing zinc which comprises maintaining an unbroken surface of a molten bath of zinc with which zinc vapors contact and on which the vapors condense and maintaining the surface bright by a surface flow from one end to the other of the bath. 40

2. The process of condensing zinc which comprises maintaining a plurality of successive baths of molten zinc, the surfaces of which are maintained unbroken and are contacted by the vapors of zinc and maintaining the surface of each bath bright by a surface flow from one end to the other thereof. 45

3. Method for condensing vapors of zinc and other volatile metals, which consists in effecting the condensation of the vapors exclusively by contact with the bright metallic surface of a bath of liquid metal, the bulk of which is sufficiently large to equalize any slight variation of the proper condensation temperature and said temperature being maintained by regulating the temperature 50 of the metal bath proper, while the temperature of other interior surfaces of the condenser is kept above the condensation temperature. 55

In witness whereof I affix my signature.  
FILIP THARALDSEN.